

# UNITED STATES PATENT OFFICE.

JAMES F. O'BRIEN, OF CHICAGO, ILLINOIS.

## EXPLOSIVE.

1,038,187.

Specification of Letters Patent. Patented Sept. 10, 1912.

No Drawing.

Application filed September 5, 1911. Serial No. 647,474.

*To all whom it may concern:*

Be it known that I, JAMES F. O'BRIEN, a citizen of the United States, residing at Chicago, in the county of Cook, State of Illinois, have invented new and useful Improvements in Explosives, of which the following is a specification.

This invention relates to an explosive which may be regarded as a derivative of an explosive for which I have filed application for United States Letters Patent on September 5th, 1911, bearing Serial No. 647,473; and the present invention consists in certain changes and additions to the formulæ there-  
in set forth for the purpose of producing an explosive greatly cheaper in manufacture and only slightly inferior in explosive quality.

In the application above referred to I have described as a basis for that explosive a mixture of a chlorate of an alkali metal and a carbo-hydrate in approximate proportion three to one. This mixture forms the basis of the explosive of this application; and the main difference between this and the other explosive is the addition of a certain amount of silico-aluminous material, such as finely powdered brick dust, to form an inert body for the explosive and to reduce its cost of manufacture. But, while reducing the cost of manufacture, the insertion of this comparatively inert substance does not reduce the explosive energy of the powder in the same ratio; so that, value for value, this powder of the present application will do more work than the powder of the application above referred to.

In its specific and most preferred form my present explosive consists of potassium chlorate about sixty per cent., sugar about eighteen per cent., starch about two per cent., and finely pulverized brick dust about twenty per cent. The proportion of brick dust may be increased to as much as thirty-five or forty per cent. of the whole weight, thereby decreasing the weight of the chlorate and of the carbo-hydrate. But the weight of the chlorate and the carbo-hydrate is most efficiently kept at the ratio of approximately three to one. The amount of sugar or of starch may be varied providing the total of carbo-hydrate be kept at approximately one-third the weight of the chlorate. Thus, I may utilize ten per cent. of starch and ten per cent. of sugar together

with sixty per cent. of the chlorate. Other carbo-hydrates may be used, these being taken as typical and as very efficient.

In the manufacture of this explosive the sugar is first dissolved or wetted and then melted. The powdered chlorate and the pulverized brick dust are mixed together and the sugar is then mixed with this mixture. The starch or other carbo-hydrate is mixed with the sugar before being mixed with the other ingredients or the ingredients may all be mixed together at one time. After mixing, the mass is dried and suitably granulated.

In order to control the speed of combustion of this explosive, as in the explosive of the application above referred to, I may utilize a small amount of ferric ferrocyanid up to approximately a maximum of two per cent. of the whole explosive. This cyanogen compound may be mixed with the sugar before the sugar is mixed with the other ingredients or it may be placed in the mixture while they are being mixed together. The cyanogen compound has the effect of increasing the speed of combustion as more is added to the explosive; two pounds of the cyanogen compound in two thousand pounds of the explosive renders the powder extremely quick in combustion, resembling the explosion of dynamite or nitro glycerin. Without any of the cyanogen compound, or with a very small amount, the combustion is comparatively slow and the powder is adapted particularly for work in soft materials where it is desired not to blast them into small pieces.

The explosive as above described has the advantage of being extremely simple in composition and preparation and of very low manufacturing cost. The addition of the brick dust (calcined clay) greatly reduces the manufacturing cost without proportionately reducing the explosive energy. Although the brick dust is a comparatively inert substance, I have found that it adds materially to the explosive energy of the explosive. That is, the addition of a certain amount of calcined clay to a certain mass of carbo-hydrate and chlorate will increase the explosive energy of the mass, but will somewhat decrease its explosive energy per unit mass. The amount of brick dust may be varied to suit conditions; for ordinary purposes about twenty

per cent. of the weight of other ingredients is found desirable. The action of the clay is ascribed to the silicates of aluminum therein present in varying proportions. The silicates seem to react with potassium and chlorin to liberate oxygen, this reaction being borne out by the fact that explosion of a mixture without the silicate material will leave a small white deposit of potassium chlorid, while the explosion of a mixture with the silicate material leaves no such residue.

Having described my invention, I claim:

1. An explosive, consisting of a chlorate of an alkali metal, a carbo-hydrate, and a silico-aluminous substance.
2. An explosive, consisting of a chlorate of an alkali metal, a carbo-hydrate, and a comparatively inert substance containing silico-aluminous material.
3. An explosive, consisting of a chlorate of an alkali metal and carbo-hydrate in the approximate proportions three to one, and a silico-aluminous substance.
- 25 4. An explosive, consisting of a chlorate of an alkali metal, a carbo-hydrate, and finely divided burned clay.
5. An explosive, consisting of a chlorate of an alkali metal and carbo-hydrate in the approximate proportions three to one, and finely divided burned clay.
- 30 6. An explosive consisting of  $KClO_3$  sixty per cent. and  $C_{12}H_{22}O_{11}$  and  $C_6H_{10}O_5$  together twenty per cent. and brick dust twenty per cent.
7. An explosive, consisting of  $KClO_3$  sixty per cent. and  $C_{12}H_{22}O_{11}$  and  $C_6H_{10}O_5$  together twenty per cent., a relatively small amount of  $Fe_4[Fe(CN)_6]_3$ , and brick dust twenty per cent.
- 40 8. An explosive, consisting of a chlorate of an alkali metal and carbo-hydrate in the approximate proportions three to one, finely divided burned clay, and a cyanogen compound.
9. An explosive, consisting of a chlorate of an alkali metal, a carbo-hydrate, a silico-aluminous substance, and a cyanogen compound.
10. An explosive, consisting of a chlorate of an alkali metal, a carbo-hydrate of the sugar group, and a silico-aluminous substance.
11. An explosive, consisting of a chlorate of an alkali metal, a sugar, and a silico-aluminous substance.
12. An explosive, consisting of potassium chlorate, sugar, and finely divided burned clay.

In witness that I claim the foregoing I have hereunto subscribed my name this 30th day of August, 1911.

JAMES F. O'BRIEN.

Witnesses:

JAS. H. BALLAGH,  
JAMES T. BARKELEW.

Copies of this patent may be obtained for five cents each, by addressing the "Commissioner of Patents, Washington, D. C."